

## UNITED STATES PATENT OFFICE

2,158,836

PRODUCTION OF LIGHT-SENSITIVE  
DIAZOTYPE LAYERS

Maximilian Paul Schmidt and Georg Werner,  
Wiesbaden-Biebrich, Germany, assignors to  
Kalle & Co. Aktiengesellschaft, Wiesbaden-  
Biebrich, Germany

No Drawing. Application March 27, 1937, Serial  
No. 133,384. In Germany April 22, 1936

9 Claims. (Cl. 95—7)

The present invention relates to the production of light-sensitive diazotype layers.

Of the diazo-compounds proposed for the positive diazo-type process only the diazo-compounds of the o-aminonaphthols and p-diamines have been able to attain any considerable practical importance. These diazo-compounds are very light-sensitive, possess good lasting properties and are more or less coloured. Moreover they fade during the exposure, so that a good white ground is obtained, and, when suitable azo-components are employed, they give dark colour tones.

The employment of other previously proposed coloured and stable diazo-compounds is open in part to the objection that their light-sensitivity is low or that they do not fade sufficiently, which gives rise to prints having poor contrast. In particular, with the compounds in question the desired dark and strong colour tones are generally not obtained.

It is an object of the invention to produce new diazotype layers of high technical value. These layers can be applied in the usual manner on or in a suitable support.

25 It has been found that light-sensitive layers containing a diazo compound of a para-aminodiphenyl which carries in the nucleus carrying the diazo group two alkoxy groups in 2- and 5-positions can be employed exceptionally advantageously for the diazotype process. The diazo compound of 4-amino-2,5-diethoxydiphenyl is a compound of this kind. The designations 1- or 1'-position, respectively, in this specification indicate the places at which the benzene nuclei of 30 the diphenyl are combined with one another. As alkyl groups in the alkoxy groups, methyl and ethyl are of particular value. The alkyl groups may also be propyl or butyl groups. Alkyl residues of higher molecular weight are less suitable. 35 The compounds named are highly coloured, lasting and of good light-sensitivity and they give, even when the ordinary azo coupling components—for example, phloroglucine—are employed, dark colour tones which are fast to light. 40 The new diazo-compounds generally couple rather energetically, so that they are particularly suitable for the wet diazotype process. They may, however, also be applied to a base together with azo-components which couple more slowly, 45 such as, for example, naphthol sulphonic acids. Layers are then obtained which can be developed either by the dry process with ammonia, or by the wet process, for example with soda solution. In certain circumstances a paper containing the 50 diazo-compound—if desired, together with an

azo-component—may have the developing substances rubbed on to it in powder form. The layers thus obtained only require for their development a treatment with steam.

Good results are in particular obtained with such compounds as contain in addition also ether groups in the other benzene nucleus preferably in 4'-position, such as, for example the diazo-compound of 4-amino-2,5-diethoxy-4'-methoxy-diphenyl. As ether groups in the nucleus containing no diazo group methoxy-and-ethoxy groups are particularly suitable. In place of these groups also a methyl group can be employed. Such bodies substituted in both nuclei give particularly deeply coloured layers, so that when copying the formation of the image can be very readily followed. The layers may be exposed by the aid of the various customary sources of light. If desired, still further substituents, such as alkyl groups or halogens, may be introduced into the molecule of the diazo-compound, whereby the colour tones are more or less altered.

Examples of some preferred methods of carrying the invention into practice are set forth below:

(1) A 3% aqueous solution of the diazo-compound of 4-amino-2,5-diethoxydiphenyl



which for the purpose of stabilization also contains a suitable acid, such as tartaric acid or boric acid, and, if desired, a means for preventing yellowing, is painted on to a base of the usual kind and is exposed behind a pattern. By development with a weakly alkaline phloroglucine solution, for example a solution containing sodium acetate, prints with brownish black lines are obtained.

(2) 31 grammes of the hydrochloride of the diazo-compound of 4-amino-2,5,4'-trimethoxydiphenyl, 10 grammes of tartaric acid, 10 grammes of boric acid, 40 grammes of thiourea, 10 grammes of ammonium sulphate and 15 grammes of aluminium sulphate are dissolved in 1 litre of water. With this solution a suitable base is coated, a deep orange-yellow coloured layer of high light-sensitivity being obtained. For the development of the exposed layer a solution containing 60 grammes of di-sodium phosphate, 80 grammes of tri-sodium citrate, 4 grammes of phloroglucine and 15 grammes of acid sodium

tartrate in 1000 c. c. of water is employed. Prints with beautiful black lines are thus obtained. If desired, other developers, which are somewhat more strongly alkaline or which contain other 5 coupling components, may also be used.

(3) 15 grammes of the zinc salt of the diazo-compound of 4-amino-2,5-diethoxy-4'-methyldiphenyl, 20 grammes of tartaric acid, 50 grammes of sodium naphthalene trisulphonate and 20 grammes of sodium 1-naphthol-4,7-disulphonate 10 are dissolved successively in 1000 c.c. of water and coated on paper. After exposure behind a pattern the prints can be developed with ammonia gas or by the application of a weakly alkaline 15 solution, which, for example, may contain sodium acetate or sodium bicarbonate.

(4) 30 grammes of the hydrochloride of the diazo-compound obtained from 4-amino-2,5-diethoxy-4'-acetylaminodiphenyl, 20 grammes of citric acid, 5 grammes of boric acid, 10 grammes of ammonium sulphate, 10 grammes of aluminium sulphate, 10 grammes of thiourea are dissolved in 1000 c.c. of water. Paper coated with this solution is exposed after drying beneath a pattern. 25 For the development a solution of 20 grammes of phloroglucine, 20 grammes of sodium acetate and 10 grammes of sodium bicarbonate in 1000 c.c. of water is employed. Prints with dark brown lines are obtained.

(5) 20 grammes of the chlorhydrate of the diazo-compound of 4-amino-2,5,4'-triethoxydiphenyl, 2 grammes of sodium bisulphate, 40 grammes of tartaric acid, 40 grammes of aluminium sulphate, 40 grammes of citric acid and 40 g. 35 of thiourea are dissolved in 1000 c.c. of water in the stated succession. With this solution a suitable support as for instance paper or cellulosehydrate foil is coated or impregnated respectively. The dried material is developed after exposing 40 with a solution of 20 grammes of phloroglucine and 40 grammes of sodium bicarbonate in 1000 c.c. of water. Prints with black-brown lines are obtained. Instead of the mentioned diazo-compound also the diazo-compound of 4-amino-2,5,5'-45 triethoxydiphenyl or the diazo-compound of 4-amino-2,5-diethoxy-4'-methoxydiphenyl may be employed.

(6) 20 grammes of the hydrochloride of the diazo-compound obtained from 4-amino-2,5-di-n-butoxy-4'-ethoxydiphenyl, 40 grammes of tartaric acid, 20 grammes of thiourea are dissolved in 50 water in the stated succession. Paper is coated with this solution. The development of the material may be effected by means of a developer,

which contains 20 grammes of phloroglucine and 40 grammes of sodium acetate in 1000 c.c. of water. The lines of the obtained prints are black-blue.

We claim:

1. Light-sensitive layer comprising the mono-diazo compound of a 4-amino-2,5-dialkoxydiphenyl, which contains in the nucleus containing no diazo group a substituent selected from the group consisting of the methyl group, the methoxy group and the ethoxy group. 5

2. Light-sensitive layer comprising the mono-diazo compound of a 4-amino-2,5-dialkoxydiphenyl, which contains in the nucleus containing no diazo group in the 4'-position a substituent selected from the group consisting of the methyl group, the methoxy group and the ethoxy group. 10

3. Light-sensitive layer comprising the mono-diazo compound of 4-amino-2,5,4'-trimethoxydiphenyl. 15

4. Light-sensitive layer comprising the mono-diazo compound of 4-amino-2,5,4'-triethoxydiphenyl. 20

5. Light-sensitive layer comprising the mono-diazo compound of 4-amino-2,5-diethoxy-4'-methoxydiphenyl. 25

6. Light-sensitive layer comprising the mono-diazo compound of a p-aminodiphenyl which carries in the nucleus containing the diazo group two alkoxy groups in 2- and 5-positions. 30

7. Light-sensitive layer comprising the mono-diazo compound of a p-aminodiphenyl which carries in the nucleus containing the diazo group two alkoxy groups in 2- and 5-positions wherein the said alkoxy groups contain one to four carbon atoms. 35

8. Light-sensitive layer comprising the mono-diazo compound of a 4-amino-2,5-dialkoxydiphenyl wherein the said alkoxy groups contain one to four carbon atoms, the diazo compound carrying in the nucleus containing no diazo group a substituent selected from the group consisting of the methyl group, the methoxy group and the ethoxy group. 40

9. Light-sensitive layer comprising the mono-diazo compound of a 4-amino-2,5-dialkoxydiphenyl wherein the said alkoxy groups contain one to four carbon atoms, the diazo compound carrying in the nucleus containing no diazo group, in the 4'-position, a substituent selected from the group consisting of the methyl group, the methoxy group and the ethoxy group. 45

MAXIMILIAN PAUL SCHMIDT.  
GEORG WERNER.